

# UNITED STATES PATENT OFFICE.

FREDERICK M. BECKET, OF NIAGARA FALLS, NEW YORK, ASSIGNOR TO UNION CARBIDE COMPANY, OF NEW YORK, N. Y., A CORPORATION OF VIRGINIA.

## MANUFACTURE OF CALCIUM CARBIDE.

1,137,567.

No Drawing.

Specification of Letters Patent. Patented Apr. 27, 1915.

Application filed January 20, 1915. Serial No. 3,384.

To all whom it may concern:

Be it known that I, FREDERICK M. BECKET, a subject of the King of Great Britain, residing at Niagara Falls, in the county of Niagara and State of New York, have invented certain new and useful Improvements in the Manufacture of Calcium Carbide, of which the following is a specification.

This invention relates to the manufacture of calcium carbide, and particularly to an improved process of preparing the charge for reduction in the electric furnace.

It has heretofore been customary in this art to smelt a loose mixture of lime and carbon, in more or less finely-divided condition; and also to briquet mixtures of this kind in order to allow a more ready escape of the reaction gases and to avoid the formation of dust. In such briquetting processes, the lime is usually mixed with coke, charcoal, anthracite or other form of fixed carbon in substantially the proportions required for the carbide-forming reaction, together with the minimum necessary proportion of a suitable binder, usually a hydrocarbon or a carbohydrate. The briquets are formed under high pressure, baked if necessary to increase their strength, and smelted down in an electric furnace. Such briquetting processes are of course highly expensive.

According to the present invention, the charge is agglomerated into mechanically strong aggregates (that is to say, aggregates which are sufficiently resistant to crushing to adapt them for use in the largest furnaces), without resorting to briquetting or molding operations of any kind. The aggregates formed are usually irregular in shape and size, but have proven excellently adapted for furnacing, yielding a commercial grade of carbide, affording an excellent distribution of the reaction gases, and a nearly dustless operation.

An example of the invention is as follows: Calcined limestone is mixed directly with a definite proportion of a suitable bituminous coal rich in volatile matter, and the mixture is subjected to a coking operation, preferably in coke ovens of the so-called by-product type. In order, under these conditions, to obtain aggregates suitable for furnacing, it has been found necessary that certain definite conditions should be observed. In

the first place, the quantity of carbon remaining in association with the lime after the coking operation should be substantially that required for the carbide-forming reaction:—



In the second place, the quantity and nature of the bituminous matter which was associated in the original coal with the above-specified quantity of fixed carbon, must be such as to yield, without the necessity of heavy pressures, the mechanically strong aggregates above described. It will be understood therefore that coal having a rather definite character and composition must be used, although some variation from a fixed standard is permissible. In practice, I have been able to obtain excellent results with grades of bituminous coal containing from about 30 per cent. to about 36 per cent. of volatile hydrocarbons. It may be practical to employ coals containing a somewhat lower percentage of volatile hydrocarbons, say from 26 per cent. upward. In the practice of the process, I have successfully used a coal from the Youghiogheny district in Pennsylvania, which contained, after drying:—

|                 |         |    |
|-----------------|---------|----|
| Volatile matter | 35.84%  | 60 |
| Fixed carbon    | 53.77%  | 65 |
| Ash             | 10.39%  | 70 |
| Total           | 100.00% | 75 |

Moisture as received 1.60% 80

The above coal was mixed with freshly burned lime in the proportion of 110 parts of coal to 100 parts of lime, and the mixture was coked in by-product coke ovens of the regular type, the gas, tar, and ammonia being collected as in the usual coking process. The evolved gas was burned for the coking and proved to be sufficient in quantity for this purpose. After coking, the resulting mass is crushed to lumps, which may be about the size of the fist or larger, and these lumps are preferably conveyed while still hot to the electric furnace. The aggregates thus prepared are mechanically strong, and will endure considerable weathering without material injury, although the coked

mass cannot be fully quenched with water, as in ordinary coking, as it would then disintegrate. It is found that the aggregates are somewhat stronger if the coking is so conducted as to leave some three to four per cent. of volatile matter, but they usually possess sufficient strength even after the volatile matters have been expelled with substantial completeness.

- 10 In preparing the mixture for coking it is preferred to grind the lime and coal to pass a one-eighth inch mesh, and it is desirable that the ground material should be very intimately mixed. Coarser ground materials, 15 say one-fourth inch and larger, do not form an equally strong aggregate. In case coal which is very rich in bituminous matter is available, it is in some cases possible or practicable to add to the charge before coking, a 20 relatively small proportion of carbonaceous matter, such as coke or anthracite, which is high in fixed carbon, and low in bituminous matters. It would also be possible, in case 25 the bituminous coal were too poor in bituminous matter to yield aggregates of the necessary strength and resistance to crushing, to add relatively small quantities of another binder, usually bituminous in character. Such bituminous additions are however 30 never necessary in practice, since satisfactory grades of coal are easily obtained. It will be observed that in accordance with the present invention, the bituminous coal serves as the principal or predominating 35 source of supply for both the fixed carbon and the coking binder.

The present process is distinctively advantageous as applied to the production of calcium carbide, as distinguished from other reduction processes. This is primarily due to the relatively very high proportion of fixed carbon which is necessary for the carbide-forming reaction, as compared with processes for the reduction of metals. Thus 45 the reaction:



requires a proportion of fixed carbon equal to about 64 per cent. of the lime used, 50 whereas the reaction involved in the reduction of silica



requires a quantity of fixed carbon amounting only to about 40 per cent. of the silica. Similarly in the reduction of iron oxid according to the equation—



- 60 the proportion of fixed carbon theoretically required amounts to only about 22.5 per cent. of the iron oxid. It is this high proportion of fixed carbon required by the calcium-carbide-forming reaction which renders 65 it practicable, in this specific case, to supply,

with the fixed carbon contained in a suitable bituminous coal, a sufficient quantity of bituminous matter to yield under ordinary coking conditions the firm and strong aggregates suitable for furnacing.

Among the general advantages of the present process may be mentioned the following: The resulting mixture has been found to have a decidedly higher electrical resistance, under the furnacing conditions, 70 than the ordinary mixtures of lump lime and lump coke; from which it follows that with a given voltage the electrodes may be more deeply buried in the charge, thereby conserving a large amount of heat; or if desired, higher voltages may be successfully employed in the furnace, which is a very material advantage, especially in the case of 75 large furnaces, as the higher voltage gives a higher power factor. This also means that 80 the present mixture permits the use, (with a given power factor) of larger furnaces than could otherwise be employed. There is also the advantage of being able to operate at a higher frequency on a given power 85 factor, or of improving the power factor at a given frequency. The foregoing are very decided practical advantages as compared with the use of compressed or molded briquets, the conductivity of which is relatively 90 high. The process is also advantageous in that it secures all the advantages of intimate mixing, with the resulting higher 95 yields, and lessened wear on the electrodes, without the disadvantage of using a powdered mixture in the furnace. The method is furthermore economical, inasmuch as the coking is carried out under standard methods, and requires even less time per unit 100 of volume than is necessary for the coking of the coal alone.

I claim:

1. In the manufacture of calcium carbide, the process of preparing aggregates suitable for furnacing, which consists in mixing lime and a suitable coking coal in such proportions that the fixed carbon of the coal will substantially suffice for the carbide-forming reaction, said coal being sufficiently rich in bituminous matter to yield with the lime, in the proportions stated and under ordinary coking conditions, a mechanically strong aggregate suitable for furnacing, and then 115 coking said mixture.

2. In the manufacture of calcium carbide, 120 the process of preparing aggregates suitable for furnacing, which consists in mixing lime and a suitable coking coal containing nitrogen in such proportions that the fixed carbon of the coal will substantially suffice for the carbide-forming reaction, said coal being sufficiently rich in bituminous matter to yield with the lime, in the proportions stated 125 and under ordinary coking conditions, a mechanically strong aggregate suitable for 130

furnacing, and then coking said mixture in a by-product oven and collecting the volatile products, including ammonia.

3. The process of making calcium carbide, which consists in mixing lime and a suitable coking coal in such proportions that the fixed carbon of the coal will substantially suffice for the carbide-forming reaction, said coal being sufficiently rich in bituminous matter to yield with the lime, in the proportions stated and under ordinary coking

conditions, a mechanically strong aggregate suitable for furnacing, coking said mixture, and thereafter embedding electrodes within a charge of said mixture and smelting said charge to produce calcium carbide.

In testimony whereof I affix my signature in presence of two witnesses.

FREDERICK M. BECKET.

Witnesses:

F. B. MORGAN,  
D. BURGESS.